

W. E. GREENAWALT.

ELECTROLYTIC PROCESS.

APPLICATION FILED JAN. 19, 1914. RENEWED DEC. 26, 1918.

1,314,742.

Patented Sept. 2, 1919.

2 SHEETS—SHEET 1.



FIG 1



FIG 2

Witnesses

Fred L. Scott  
Jno. J. Styer.

Inventor  
William Greenawalt.

W. E. GREENAWALT.

ELECTROLYTIC PROCESS.

APPLICATION FILED JAN. 19, 1914. RENEWED DEC. 26, 1918.

1,314,742.

Patented Sept. 2, 1919.

2 SHEETS—SHEET 2.



FIG 3



FIG 4

Witnesses

Fred L. Scott  
Ino. J. Styer.

Inventor

William E. Greenawalt

# UNITED STATES PATENT OFFICE.

WILLIAM E. GREENAWALT, OF DENVER, COLORADO.

## ELECTROLYTIC PROCESS.

1,314,742.

Specification of Letters Patent.

Patented Sept. 2, 1919.

Application filed January 19, 1914, Serial No. 812,951. Renewed December 26, 1918. Serial No. 268,415.

To all whom it may concern:

Be it known that I, WILLIAM E. GREENAWALT, a citizen of the United States, residing in the city and county of Denver and the State of Colorado, have invented certain new and useful Improvements in Electrolytic Processes, of which the following is a specification.

This invention relates to improvements in electrolytic processes and has for its more immediate object the more effective application of reducing gases during electrolysis. The process will be described more particularly to the electrolysis of impure copper sulfate solutions, although it is not intended to limit it to this use alone.

In the electrolysis of impure copper sulfate solutions, as for example those obtained in leaching copper ores, there is always present iron sulfate, which injuriously affects the operation. Ferrous sulfate is not particularly harmful in the electrolyte, but the ferric sulfate is highly detrimental.

If a solution of copper sulfate, containing ferrous sulfate, is electrolyzed, copper is deposited at the cathode while sulfuric acid and ferric sulfate are produced at the anode, as represented by the following equations:



The ferric sulfate, finding its way back to the cathode, combines with the deposited copper and is again reduced to the ferrous condition, thus representing a loss of efficiency, as represented by equation:



If, however, the ferric sulfate can be reduced at the expense of a cheap reducing agent, such as sulfur dioxide, then acid is regenerated and the iron in the electrolyte loses its ability to combine with the deposited copper, as shown by equation:



so that for every molecule of iron that is reduced from the ferric to the ferrous condition two molecules of acid are regenerated. This acid is beneficial in the electrolyte, and on leaving the electrolyzer is further available for the extraction of copper from the ore.

55. Similarly, if there is an excess of sulfur

dioxide in the electrolyte, it acts as a depolarizer and acid generator, thus:



The effectiveness of these reactions and the practical results obtained, depends upon the thoroughness with which the sulfur dioxide is brought in contact with the electrolyte. In my process this is effectively and continuously accomplished, as will now be explained by referring to the accompanying drawings, in which

Figure 1 represents a plan through the apparatus illustrating the process;

Fig. 2, the corresponding longitudinal section;

Fig. 3, the plan of a modified apparatus, and

Fig. 4, the corresponding section.

In the figures, 1 is a tank containing the electrolyte, which may be presumed to be copper sulfate solution as obtained, say, from leaching copper ores. 2 are the anodes, and 3 the cathodes, 4 is a frame having stirring bars 5 interposed between the electrodes, preferably oscillating as a whole, and suspended from fixed pivotal points 6, and actuated by the mechanism 7.

10 represents the mechanism, taken as a whole, by means of which reducing gases, such as sulfur dioxide, are brought to a minute state of subdivision, or atomized, in contact with the electrolyte, and consists, preferably, of an outer tank 9, into which the electrolyte flows from the cell through the pipe 8. Inserted within the tank 9, is a tube 11, having perforated disks 12, and is suspended within the tank by the shaft 13 from the ball bearings 14. This tube is made to revolve at a high speed, being driven by the pulley 15, and the motor 16. The reducing gas, say, sulfur dioxide, is produced in the generator 17, and by means of the air or gas pump 18, is forced through the pipe 19, and into the tube 11, of the atomizer, 10. 20 is the return pipe for the reduced solution, and 21 the exhauster for the excess gas, and air or nitrogen, through the pipe 22, to prevent it from getting into the cell room and contaminating the atmosphere. Or the excess gas may be forced through another apparatus in connection with another cell.

To operate the process, the electrolyte may be presumed to be charged into the cell

1, in a reduced condition, and containing perhaps a small excess of sulfur dioxid. The oscillating frame 4 brings the soluble gas and reduced electrolyte in contact with 5 the electrodes. At the cathode the electrolyte is moved in sufficient volume to avoid the injurious formation of hydrogen except at very high current densities. At the anode the gas and reduced electrolyte is acted upon 10 by the released oxygen, and may act as a depolarizer. If the action at the anode were allowed to continue the reducing agent would soon be exhausted and the iron oxidized to the ferric condition, which would 15 be highly injurious and greatly reduce the current efficiency. To avoid this a portion of the electrolyte is allowed to flow into the atomizer 10 while at the same time the reducing gas from the generator 17, is forced 20 into the tube 11, which is revolved at a high speed, so that the gas ascending through the tube 11, and perforated disks is divided into minute particles, or atomized, in contact with the solution, and thoroughly incorporated 25 with it, thus making it possible to quickly, effectively, and continuously reduce the solution, and if desired, charge it with an excess of the gas. It is then again returned, preferably though not necessarily, 30 in a continuous stream to the electrodes. In this way the injurious ferric compounds are kept at a minimum or entirely avoided. The gas ascending through the tube 11, acts as an air lift, thus making it possible 35 to return the reduced electrolyte at a higher level than the level of the electrolyte at the electrodes. The circulation may thus be accomplished by gravity and by the buoyant action of the atomized gas in the liquid.

40 Reducing gases, such as sulfur dioxid, are only slightly soluble in water, but by the arrangement of the present process this difficulty is overcome since the gas may be continuously applied to the electrolyte and the 45 accumulation of the injurious ferric compounds, in injurious amounts, prevented.

As a modified arrangement, shown in Figs. 3 and 4, the atomizer might be inserted in the electrolyte tank 1, in a space reserved in 50 the cell for the purpose. In either case a portion of the electrolyte is temporarily segregated from the electrodes and from the main body of the electrolyte and treated with the reducing gases and then again returned 55 to the electrodes.

The process permits of considerable generation of acid and the retaining of the acid in the electrolyzer to a much greater extent than is ordinarily possible. This is a highly 60 desirable feature, as the increased acidity, and to a certain extent the accompanying increased temperature also, greatly reduces the electromotive force required for the deposition of the copper. The excess regeneration 65 of acid is also desirable as a solvent of

copper from the ore, since more acid can be then wasted without detriment and the electrolyte kept in a higher state of purity, and consequently of efficiency.

The process presents marked advantages 70 over methods in which the reducing gases are introduced into the electrolyte in contact with the electrodes, since it permits of intimate mixture of the gas and electrolyte due to the finely divided state of the 75 gas and the violent agitation of the electrolyte. It also makes it possible to exhaust the excess gas, and thus make the process workable.

The oscillation of the frame between the 80 electrodes brings the reduced electrolyte effectively in contact with the electrodes as rapidly as it is reduced, and this action is made more effective by the circulation of the electrolyte. In Fig. 4 the circulation is 85 made more effective by introducing the gas into one end of the pipe 30, thus acting as an injector, and taking the electrolyte from the further end of the cell, while the reduced electrolyte flows in the opposite direction. 90

The effective depolarization brought about by this process by the use of sulfur dioxid and ferrous sulfate produces large quantities of acid, reduces the E. M. F. for the deposition of the copper, and greatly prolongs the life of the insoluble anodes. The 95 life of the anodes depends largely on the effectiveness of the depolarization.

I claim:

1. An electrolytic process which consists 100 in electrolyzing copper solutions containing ferrous salts to deposit the copper at the cathode with a simultaneous oxidation of the ferrous salts to the ferric salts at the anode, agitating the electrolyte, segregating 105 a portion of the electrolyte from the electrodes, applying to the segregated electrolyte a gas capable of reducing the ferric salts to the ferrous condition so as to rise through the electrolyte by its own buoyancy 110 in the liquid, atomizing the gas in contact with the electrolyte as it ascends through the liquid, and returning the reduced electrolyte to the electrodes.

2. An electrolytic process which consists 115 in electrolyzing copper solutions containing ferrous salts to deposit copper at the cathode with a simultaneous oxidation of the ferrous salts to the ferric salts at the anode, segregating a portion of the electrolyte from 120 the electrodes, applying to the segregated electrolyte a gas capable of reducing the ferric salts to the ferrous condition so as to rise through the electrolyte by its own buoyancy in the liquid, atomizing the gas in contact 125 with the electrolyte as it ascends through the liquid, and returning the reduced electrolyte to the electrodes.

3. An electrolytic process which consists 130 in electrolyzing copper solutions containing

ferrous salts to deposit copper at the cathode with a simultaneous oxidation of the ferrous salts to the ferric salts at the anode, withdrawing a portion of the electrolyte 5 containing ferric salts from the electrolyzer and introducing it into a reducing chamber, applying a gaseous reducing agent to the segregated portion of the electrolyte to rise through the liquid by its own buoyancy in 10 the liquid, atomizing the gas in contact with the segregated electrolyte as it ascends through the liquid whereby the ferric salts is again reduced to the ferrous condition, and circulating the electrolyte between the 15 electrolyzer and the reducing chamber by the buoyant action of the atomized gas in the electrolyte in the reducing chamber.

4. An electrolytic process which consists in electrolyzing copper solutions containing 20 ferrous salts to deposit the copper at the cathode with the simultaneous oxidation of the ferrous salts to the ferric salts at the anode, segregating a portion of the electrolyte from the electrodes, applying sulfur di- 25 oxid to the segregated electrolyte to reduce the ferric salts to the ferrous condition and in such a way as to rise through the electrolyte by its own buoyancy in the liquid, atomizing the gas in contact with the electrolyte as it ascends through the liquid, and returning the reduced electrolyte containing 30 an excess of the gas to the electrodes.

5. An electrolytic process which consists in electrolyzing copper solutions containing 35 ferrous salts to deposit the copper at the cathode with the simultaneous oxidation of the ferrous salts to the ferric salts at the anode, applying a reducing gas to a pool of the electrolyte in a reducing chamber, 40 maintaining a flow of gas in the reducing chamber, subdividing the gas in the electrolyte in the reducing chamber, and exhausting the excess gas from the reducing chamber of one electrolyzer and applying it to 45 the electrolyte in the reducing chamber of another electrolyzer.

6. An electrolytic process which consists in electrolyzing copper solutions containing ferrous salts to deposit the copper at the 50 cathode with the simultaneous oxidation of the ferrous salts to the ferric salts at the anode, segregating a portion of the electrolyte from the electrodes into a reducing chamber, applying a reducing gas to the 55 electrolyte in the reducing chamber to reduce the ferric salts to the ferrous salts, subdividing the gas in the reducing chamber, and applying a stream of gas to a stream of

the electrolyte in such a way as to cause a flow of electrolyte into contact and out of 60 contact with the electrodes.

7. An electrolytic process which consists in electrolyzing copper solutions containing salts of iron to deposit the copper at the cathode with the simultaneous oxidation of 65 the ferrous salts to the ferric salts at the anode, segregating a portion of the electrolyte from the electrodes into a reducing chamber, applying a reducing gas to the segregated electrolyte so that it will rise 70 through the electrolyte by the pressure of the liquid on the gas, thus causing a higher liquid level in the reducing chamber than in the electrolyte tank, subdividing the gas in its ascent through the segregating electrolyte in the reducing chamber, and maintaining 75 a continuous flow of reduced electrolyte from the reducing chamber to the electrodes and of oxidized electrolyte from the electrodes to the reducing chamber. 80

8. An electrolytic process which consists in electrolyzing copper solutions containing salts of iron to deposit the copper at the cathode with the simultaneous oxidation of the ferrous salts to the ferric salts at the 85 anode, maintaining a continuous flow of electrolyte from the electrolyzer to a reducing chamber, applying a reducing gas to the lower portion of the electrolyte in the reducing chamber so that it will rise through 90 the electrolyte by the pressure of the liquid on the gas, subdividing the gas in its ascent through the electrolyte, and maintaining the flow of electrolyte by the difference in the liquid level induced by the application of 95 the gas in the reducing chamber.

9. An electrolytic process which consists in electrolyzing copper solutions containing salts of iron to deposit the copper at the cathode with the simultaneous oxidation of 100 the ferrous salts to the ferric salts at the anode, applying a reducing gas to a pool of the electrolyte in a reducing chamber, treating the electrolyte with the gas by intimately mixing the gas with the electrolyte 105 in the pool, maintaining a flow of gas through the reducing chamber, and maintaining a flow of reduced electrolyte from the pool in the reducing chamber to the electrodes and of oxidized electrolyte from 110 the electrodes to the pool.

WILLIAM E. GREENAWALT.

Witnesses:

THOMAS S. WALTENMEYER,  
EDWIN J. CHISSELL.